

# United States Patent Office

2,980,489

Patented Apr. 18, 1961

1

2,980,489

## PROCESS OF MAKING WOOL-LIKE CELLULOSIC TEXTILE MATERIALS

Hugh C. Gulledge, Newark, Del., assignor to E. I. du Pont de Nemours and Company, Wilmington, Del., a corporation of Delaware

No Drawing. Filed Jan. 9, 1958, Ser. No. 707,857

9 Claims. (Cl. 8—117)

This invention relates to the production of novel, cellulosic materials exhibiting modified properties, and more particularly to the preparation of improved fibrous cellulosic materials adapted for use in the textile industry.

Differences in the properties of wool and cotton fibers and textiles are well known in the trade and it is well recognized that a fiber possessing the properties of cotton together with the crease resistance of wool would provide a valuable product adaptable to wide and extensive usage. For instance, such material could be advantageously employed in men's light-weight suits for summer wear while presenting an appearance comparable to the warmer woolens, and in the manufacture of women's clothes since a dressy appearance would be desirably assured for substantial periods in warm and humid weather. Although heretofore many treatments have been devised and proposed, the impartation of satisfactory crease-resistance properties to cotton fabrics while retaining other desired and essential features of the fabric has not been successfully accomplished.

Cotton and artificial cellulose derived fibers are deficient in a number of desirable properties, including wrinkle resistance, mildew resistance, abrasion resistance and non-inflammability, etc. These weaknesses are probably greatest in artificial fibers, especially regenerated cellulose type rayon, and heretofore such weaknesses have been considered to be a property fundamental to the characteristics of the textile material and not subject to change or modification even when recourse to relatively expensive treatments is had.

This application is a continuation-in-part of my copending application Serial No. 474,586, filed December 10, 1954, now abandoned.

In my copending application, novel highly useful cellulosic textile materials are disclosed which advantageously possess wool-resembling properties as well as a novel combination of other desirable characteristics, including increased liveliness, crease, mildew, abrasion and flame resistance, greater warmth and insulating characteristics, together with improved washability and high melting point. Also disclosed are novel methods for converting such inexpensive type cellulosic materials to more useful products competitive with wool and synthetic fibers such as nylon polyamide-condensation-polymer and "Orlon" acrylonitrile-addition-polymer, by treating a cellulosic material with a swelling and conditioning agent, reacting the swollen cellulosic product with a metal ester in a substantially non-aqueous environment and preferably in the presence of said agent, regenerating the cellulose product by treatment with aqueous media, and separating and recovering the improved, modified cellulosic material containing the metal of the ester in chemical combination with the cellulose from the residual organic reagents, solvents and reaction products. More specifically, the modified cellulosic product is prepared by wetting a suitable cellulosic material, such as cotton or rayon, in a substantially anhydrous organic swelling and complexing agent for cellulose, such as an amine, e.g., ethyl amine or

2

ethylene diamine. Upon desired pre-swelling, conditioning or complexing being attained, excess swelling agent is drained or otherwise removed from the swollen, complexed amine cellulose product, and it is then immersed in a solution of an anhydrous organic metal ester, especially of a metal of the fourth group of the periodic table, e.g., alkyl or aryl metal esters of the ortho type, until the metal becomes transferred from the solution to the cellulose to form a highly tendered metal ester-amine cellulose intermediate compound. This product is then separated from the organic liquid, treated with water or other aqueous media, such as water-containing organic solvents, e.g., water and alcohol solutions, or dilute aqueous media, and recovery is effected of the improved, modified material of greater usefulness which will be found to retain substantially the macroscopic shape and geometric character of the original cellulose fiber and will be crease and wrinkle resistant.

It has been found that, in accordance with this invention, products derived from the invention of my said co-pending application can be effectively and advantageously improved, particularly in respect to desired tensile strength and fade resistance properties, if in their preparation a plurality of substantially anhydrous organic metal esters, more especially mixed esters comprising those of antimony and a metal from the fourth group of the periodic table, such as titanium or zirconium, are employed.

Accordingly, it is among the objects of this invention to provide such improved, modified cellulosic products and novel methods for effecting their preparation. Particular objects of the invention include: the provision of improved stable, fibrous cellulosic materials adaptable for use in the textile field; of products exhibiting enhanced wool-like characteristics and which are crease and wrinkle resistant; the provision of a product of this character which is suitably stabilized against loss of tensile strength due to aging or photodegradation, and which is free from any obtainable tendency toward tenderizing or fading as a result of exposure to ultraviolet light. Other objects and advantages will be apparent from the ensuing description of the invention.

In practically adapting the invention, cotton, rayon or other suitable cellulosic material to be modified is subjected to wetting treatment in a substantially anhydrous, pure liquid amine conditioning agent until desired swelling thereof is effected. Excess of the amine treating agent is removed from the resulting swollen, complexed amine cellulose product, following which it is immersed for reaction at an elevated temperature in a solution of the contemplated mixed anhydrous metal esters, one of which comprises a hydrolyzable ester of antimony, e.g., alkyl or aryl metal esters of the ortho type, and until the metals of said esters become transferred from the solution to the cellulose and a highly tendered metallized ester-amine cellulose intermediate compound is formed. If desired, the metal esters can be added to the cellulose as a mixed solution in an anhydrous organic solvent, or as separate anhydrous solutions in sequential order and while the cellulose remains wetted by the conditioning agent. Preferably, the metal esters used comprise the trialkyl antimonites, such as trimethyl, triethyl, tripropyl, or tributyl antimonite, etc., or mixtures thereof, and titanium or zirconium ortho esters, such as tetraalkyl titanates or zirconates, e.g., tetramethyl, tetraethyl, tetrapropyl, tetrabutyl titanate or zirconate, etc., or various mixtures thereof. Upon formation of said intermediate compound, it is separated from the organic liquid, treated with aqueous media as contemplated in my aforementioned copending application, and recovery is then effected of the improved modified product of this invention.

To a clearer understanding of the invention, the fol-

lowing specific examples are given. These are merely illustrative and not in limitation of said invention.

#### EXAMPLE I

35 grams of 2.85 oz. boiled off cotton fabric was dried in air at 110° C. for two hours and then placed in a conventional type vessel equipped with a reflux condenser and sealed from the atmosphere through a nitrogen trap. Anhydrous monoethylamine, containing less than 1% of water, was added to cover the sample. After soaking for 1½ hours at approximately 16° C. the liquid amine was drained from the sample and a solution, comprising 730 grams of isopropanol, 490 grams of tetraisopropyl titanate and 8 grams of tributyl antimonite, was added. This solution, containing the sample, was heated at reflux temperatures for two hours and then drained. The sample was washed free of excess metal ester and amine with several portions of anhydrous isopropanol. The washing was continued until a sample of the washings showed no cloudiness upon water addition. Water at room temperature was then added to cover the fabric and the whole allowed to stand for one hour. The fabric was then removed and dried. The pertinent improved properties of this product are shown below in Table I.

#### EXAMPLE II

Example I was repeated, except that the ester containing solution comprised 750 grams of isopropanol, 500 grams of tetraisopropyl titanate, and 16 grams of tributyl antimonite. The results of this treatment are also shown in Table I below.

#### EXAMPLE III

The procedure of Example I was again duplicated, except that the titanating solution used comprised 750 grams of isopropanol, 500 grams of tetraisopropyl titanate, and 44 grams of tributyl antimonite.

The results of this treatment are also shown in the following Table I:

Table I

|                                           | Analysis of Fabric         |                                          | Relative Tear Strength After 25 Days—45° Southern Exposure, September, Grams |
|-------------------------------------------|----------------------------|------------------------------------------|------------------------------------------------------------------------------|
|                                           | TiO <sub>2</sub> , Percent | Sb <sub>2</sub> O <sub>3</sub> , Percent |                                                                              |
| Sample Untreated Control                  |                            |                                          | 1,100                                                                        |
| Sample treated with TPT only <sup>1</sup> | 13.0                       | 2.7                                      | 100                                                                          |
| Example I                                 | 13.0                       | 2.7                                      | 300                                                                          |
| Example II                                | 11.8                       | 4.3                                      | 920                                                                          |
| Example III                               | 7.4                        | 9.5                                      | 1,170                                                                        |

<sup>1</sup> As in Example I, except no antimonite was present.

(The relative tear strength data given in Table I above and Table II below were obtained as follows: a swatch of fabric, approximately 3 x 10 inches square, was cut at one end to form a one inch slit. One of the split ends was fastened to a spring scale and the other to a clamp which could be pulled away from the scale by hand. By pulling the split strip in this manner a nine inch tear was made and the load during tearing was read from the scale in grams. The difference in magnitude of the figures given in Tables I and II is due to a different type of fabric, of stronger characteristic, used in Table II.)

#### EXAMPLE IV

1/4 lb. skeins of 40/2 ply grey cotton yarn were packed in baskets and dried in an oven at 110° C. for 2 hours. The baskets containing the dried yarn were then placed in a dyeing machine and blanketed with dry nitrogen. This dyeing machine was equipped to treat the yarn with a liquid, either at atmospheric pressures or somewhat elevated pressures. Anhydrous monoethylamine was circulated through the yarn for one hour at 3° C. The free amine was drained off and 5 gallons of a solution of tetraisopropyl titanate in isopropanol, analyzing 9.1%

TiO<sub>2</sub> and containing 200 grams of triisopropyl antimonite, were added. This solution was circulated through the yarn at 60° C. for 1 1/4 hours. The nitrogen blanketing vents were then closed and the solution heated at 85° C. under 25 lbs. pressure for one hour. After cooling to 60° C., the metallating solution was drained and the excess unreacted metal esters washed out of the yarn with isopropanol at 60° C. Water at 30° C. was then added and circulated for 30 minutes. The yarn was removed, centrifuged and dried, and woven into fabric for testing. The properties of the fabric obtained are shown in Table II below.

#### EXAMPLE V

Example IV was repeated, except that the titanating solution used comprised 5 gallons of an isopropanol solution of tetraisopropyl titanate, containing 9.3% TiO<sub>2</sub>, plus 400 grams of isopropyl antimonite. Tests on the fabric treated in accordance with this example are shown in Table II below.

#### EXAMPLE VI

Example IV was repeated except that a titanating solution comprising 5 gallons of an isopropanol solution of tetraisopropyl titanate analyzing 9.6% TiO<sub>3</sub> and 700 grams of triisopropyl antimonite was used. Tests on the resulting fabric from this example are also given in Table II below.

#### EXAMPLE VII

Example IV was repeated except that a titanating solution comprising 5 gallons of an isopropanol solution of tetraisopropyl titanate analyzing 8.5% TiO<sub>2</sub> and 1400 grams of triisopropyl antimonite was used. Table II below also shows the properties of the fabric obtained in this example.

Table II

| Sample                   | Fabric Analysis            |                                          | Crease Test Percent Recovery After 300 sec. | Relative Tear Strength After 35 Days—45° Southern Exposure, March, Grams |
|--------------------------|----------------------------|------------------------------------------|---------------------------------------------|--------------------------------------------------------------------------|
|                          | TiO <sub>2</sub> , Percent | Sb <sub>2</sub> O <sub>3</sub> , Percent |                                             |                                                                          |
| Example IV               | 20.0                       | 1.8                                      | 69                                          | 900                                                                      |
| Example V                | 19.3                       | 3.8                                      | 72                                          | 1,900                                                                    |
| Example VI               | 16.5                       | 6.8                                      | 72                                          | 2,900                                                                    |
| Example VII              | 13.3                       | 11.9                                     | 68                                          | 3,200                                                                    |
| Untreated Cotton Control |                            |                                          | 54                                          | 4,200                                                                    |
| Titanated Cotton Control | 17.5                       |                                          | 69                                          | 700                                                                      |

(The crease test used in this table is designed to measure the ability of the fabric to recover from creasing or wrinkling, and is described in Technical Bulletin #T-7, published December 1, 1947 of Monsanto Chemical Company.)

#### EXAMPLE VIII

Example I was repeated, except that an ester containing solution, comprising 750 grams of isopropanol, 500 grams of tetraisopropyl zirconate and 16 grams of tributyl antimonite was employed. The final product analyzed 12% ZrO<sub>2</sub> and 4.2% Sb<sub>2</sub>O<sub>3</sub>. The relative tear strength was tested as in Examples I to III, and the product was determined to be slightly better than the titanium containing product of Example II. The modified cotton fabric was crease resistant and had wool-like properties.

#### EXAMPLE IX

A treatment similar to that carried out in Example III was effected but with a sequential contact of the fabric with a separate titanium ester solution and with a separate antimony ester solution, instead of through the simultaneous contact of a combined solution of the metal esters as used in Example III. The fabric was first immersed in a tetraisopropyl titanate solution consisting of 750 grams of isopropanol and 500 grams of the titanate and maintained therein at a temperature of 80° C. for two hours with mild agitation. Subsequently, the

fabric was removed and drained and was then immersed in a second isopropanol solution containing 44 grams of tributyl antimonite for each 750 grams of isopropanol. This treatment was also continued for two hours at 80° C. as before. The fabric was removed, rinsed with isopropanol, dried, analyzed and tested as in the instance of Example III. The results obtained were similar to those shown in Table I for the product from Example III. The fabric possessed improved crease resistant properties and relative tear strength after 25 days Southern Exposure better than the untreated control, a TiO<sub>2</sub> content of 7.6% and a Sb<sub>2</sub>O<sub>3</sub> content of 9.9%.

Although described and illustrated above as applied to certain specific embodiments, the invention is not to be considered as limited thereto. Hence, while particular temperatures, times, pressures, reactants, ratios, concentrations, etc., have been used, these can be suitably varied without departing from the spirit and scope of the invention. Thus, in the metallation step, temperatures ranging from about room (25° C.) to 150° C., or higher, and preferably from about 40° C. to 100° C. can be resorted to, as can relatively short or long, say, up to 24 hours, reaction time periods. In general, at higher temperatures, relatively short periods are required, while longer periods are necessary when lower temperatures are used, with the time and temperatures employed controlling the extent of cellulose effected. When employing relatively prolonged reaction periods at high temperatures, it will be found desirable to blanket the reactants with an inert gas, such as nitrogen, argon, helium, etc., in order to exclude oxygen or like undesired gases presence so that any tendency toward degradation of the final cellulose product will be avoided. The pressures utilized can range from atmospheric to any extent required to maintain the desired liquid condition, e.g., up to the vapor pressure of the solution, solvent, amine and metal ester mixture used at the temperature employed. Again, complexing agents especially useful herein comprise any nitrogenous swelling agent such as ammonia and amine-nitrogen compounds containing a —NH<sub>2</sub> or NH radical. Examples thereof include short chain or small ring primary or secondary mono- or poly-organic ammonia derivatives. Liquid anhydrous NH<sub>3</sub>, ethyl amine, methyl amine, ethylene diamine, and diethylene triamine are especially useful and effective. Other useful agents include hydrazine, formamide, urea, phenyl urea, thio urea, isopropyl amine, propylene diamine, triethylene tetramine, trimethylene tetramine, dimethyl amine, N-acetyl methylamine, diethylene amine; difunctional short chain amine derivatives such as ethanolamine, 1,3-diaminopropanol-2, aminoethyl ethanolamine, etc. These reactive nitrogenous reagents, known for their ability to swell cellulose, have proved effectively useful and can be used in pure state, being added to and caused to react with substantially anhydrous cellulose under pressure and temperature conditions consistent with the maintenance of a major part of the swelling and complexing agent in the liquid state. By conditioning agents I refer to those compounds, usually swelling agents, which suitably modify the cellulose and enable or promote reaction therewith of a titanium or other contemplated metal ester. Since my process is less complicated when the reagent is employed in pure, liquid state, e.g., pure methyl amine or pure ethylene diamine, I preferably resort to this form of reagent. If desired, substantially non-aqueous solutions of the reagents in compatible organic solvents can also be employed. It is preferable that the amine swelling agent and also the cellulosic material to be treated be substantially dry. However, the incidental presence of small quantities of water in either does not seriously interfere with the process as will be shown below.

The metal ester can be added as a pure liquid, or more suitably, as a solution in an organic solvent, such as an alcohol, benzene, toluene, xylene, cyclohexane,

dioxane, paraffin, hydrocarbon, etc. While tetraisopropyl titanate as a solution in isopropanol is preferred for use because it is one of the less expensive useful titanates from which economical recovery of the isopropanol can be effected, the invention is not limited thereto.

As already indicated, general use is contemplated in conjunction with an antimony ester of any hydrolyzable organic ester of a polyvalent metal, especially of Fourth Group metals, such as titanium or zirconium, or mixtures thereof adapted to tenderize swollen cellulose. This includes the ortho esters as well as the partially condensed esters. The ortho esters are defined by the formula M(OR)<sub>x</sub> in which M includes aluminum, iron (ferric), titanium, zirconium, hafnium, thorium, etc., e.g., 10 metals which form water insoluble oxides and have a coordination number at least one greater than the valence of the metal in the oxide form (which number is usually 6), R is a monovalent hydrocarbon or chlorinated hydrocarbon radical, such as an alkyl (methyl, ethyl, propyl, butyl, amyl, isopropyl, isobutyl, isoamyl, etc.), cycloalkyl (cyclopropyl, cyclobutyl, cyclopentyl, etc.) aryl (phenyl, naphthyl, etc.), alkaryl (tolyl, xylyl, ethylphenyl, propylphenyl, etc.), aralkyl (benzyl, phenylethyl, phenylpropyl, etc.), and x is 3 and 4, the valence in its highest 15 state of oxidation. For reasons of economy, esters having the smaller alkyl radicals (1-6 carbon atoms) are preferred for use, such as methyl, ethyl, propyl, isopropyl, butyl, etc. Examples thereof include the various titanium, zirconium, hafnium, thorium, aluminum, iron tetraethylates, isopropylates, butylates, hexylates, etc., as well 20 as the monochloro and dichloro derivatives of these compounds. However the various cyclohexylates, phenylates, benzylates and naphthylates, and any ester containing a hydrocarbon radical having from 1-12 carbon atoms 25 are satisfactorily useful. Chlorinated hydrocarbon radicals in this molecular weight range especially those obtained as titanates by the reaction of titanium tetrachloride upon ethylene oxide and propylene oxide are readily employable. The partially condensed titanates and zirconates usually formed by the reaction between water 30 and the ortho esters, e.g., tetraalkyl titanates, are also useful in preparing my metallated cellulose. When these condensed esters are used, it is not necessary to have absolutely dry cellulose or amine swelling agent as starting materials. The presence of, say, a fraction of a 35 percent of water in the amine solution merely acts to polymerize a portion of the ortho ester used in the metal treating step. The degree of polymerization of the esters included in this process is preferably less than that obtained by the interaction of an equimolar quantity of 40 water. Similarly useful are esters containing cycloalkyl, aryl, or aralkyl radicals, e.g., phenyl, naphthyl, benzyl, etc.

Hydrolyzable antimony organic esters contemplated for use herein in conjunction with the ortho esters mentioned 45 are variable and can comprise antimonates and antimonites. The latter, or mixtures thereof, are preferred for use and correspond to the formula (RO)<sub>3</sub>Sb, wherein R is a monovalent hydrocarbon radical, such as the various alkyls, aryls, aralkyls, cycloalkyls, mentioned above, e.g., methyl, ethyl, propyl, butyl, cyclopropyl, phenyl, naphthyl, tolyl, anthranyl, benzyl, xylyl, ethyl phenyl, phenyl propyl, etc. and the monochloro, dichloro, etc., derivatives of such compounds. Especially useful are 50 trialkyl antimonites in which the hydrocarbon radical contains from 1-12 and preferably from 1-6 carbon atoms. Examples thereof include trimethyl, ethyl, isopropyl, butyl, hexyl, octyl, benzyl, phenyl antimonites and their various mixtures. These esters are applied under substantially anhydrous conditions, although the 55 presence of small amounts of water, as indicated in connection with the titanium esters, can be tolerated. The antimony ester is preferably used in combination, that is, simultaneously with the titanium or zirconium esters, or 60 75 they may be applied sequentially, e.g., before or after the

titanating step, but prior to the water-washing step. Also, in such sequential method, I may treat the amine swollen, titanated and water regenerated cellulose with antimony by reswelling it with an amine and then treating it with an alkyl antimonite. This method serves to incorporate advantageously a maximum amount of titanium or zirconium, in the final product. Temperatures at or near the boiling temperature of the anhydrous solvent are referred to in the examples during the metallation treatment. As noted, lower temperatures may be employed and may even be preferred on commercial scale where heating and cooling equipment would be burdensome. The use of lower temperatures, say, room temperature, should be accompanied by longer contact time for the fabric and the metal ester solution.

The anhydrous metal ester is added preferably, as stated, to the cellulose while the latter is still wetted by the amine conditioning agent and the metallation is preferably carried out in the presence of such agent. The ester-amine-cellulose complex intermediate derived from reaction of the preconditioned cellulose with the ester is in severely tendered state compared to the cellulose compound resulting from the initial swelling and complexing treatment, or compared to the initial cellulose material. That is, it is characterized by lack of strength, with the fabric tensile and tear strength being substantially reduced, i.e. by about 10-90%, and usually to 10-30% of its original strength, and the tenacity of yarns or fibers being reduced to a similar extent. Upon completion of the metallation, unreacted ester, amine and solvent used are drained from the intermediate with substantially anhydrous conditions still prevailing. Removal of these unreacted materials can be further facilitated by subsequent displacement washes, using anhydrous organic solvents, followed by draining or other physical separation methods. The anhydrous solvent-washed ester-amine-complexed cellulose intermediate can be used in various applications. For example, it can be immediately placed in an aqueous medium, whereupon the hydrolysis product of the intermediate is removed to leave the metal radical in reacted condition within the cellulose structure as a cellulose derivative having substantially the strength and washability and high melting point of the original fibrous cellulose material. Advantageously, it will possess not only the increased tensile strength and photodegradation resistant properties mentioned above but the novel high flame, mildew resistance and single fiber characteristics of wool, including initial modulus, compliance ratio, work recovery, crimp elongation, and wool-like woven cloth properties, e.g., handle, high crease and wrinkle resistance shown in my said copending application. In addition, it possesses high laundering resistance, which property and the existing new chemical composition is retained even after repeated washing treatments, as is also demonstrated in the disclosure of my said copending application.

As the above examples and tables of test data show, the products from my process possess new and very desirable improvement properties. In addition to their high resistance to photodegradation and excellent wrinkle resistant and general wool-like properties, they are both flame resistant and mildew resistant, and these desirable properties are retained even after repeated launderings. This combination of properties gives new potential uses to cellulose fabrics, such as cotton and rayon. My novel treatments also provide very marked improvements in other cellulosic fibrous materials, such as linen and ramie, and renders possible the preparation of light weight comfortable summer wearing apparel from cotton and rayon, which will have wool-like properties and be resistant to degradation by sunlight.

The products of this invention will also advantageously retain substantially the macroscopic shape and geometric character of the original cellulose fiber. They will be substantially insoluble in acetone and cuprammonium

solutions. In respect to wool-like and wrinkle resistance properties alone they exhibit an at-least 20% and usually a 30% or greater improvement over untreated cotton. Prior art products give very low wrinkle resistance as measured by hand test or by the crease tester method referred to in my said copending application. Although the fibers resulting from my novel treatment have an increased fiber density value substantially as would be expected due to metallation, the bulking value, i.e., vol./wt. ratio is uniquely increased. This characteristic along with enhanced elasticity which is indicated by elongation at the break point, demonstrates that wool-like properties, in addition to crease resistance, are attained by my process.

As already indicated, it is unnecessary to effect removal of substantially all of the amine swelling agent from the cellulose prior to the metallation treatment. In fact, the presence of the amine in some concentration during such step will be found to enhance the ultimate metallation effected. Thus, for example, the metallation can be carried out with an isopropanol solution containing approximately 18% by weight of tetraisopropyl titanate, 15% of isopropyl antimonite and 15% of ethyl amine. As little as 2 or 3% of the amine will be noticeably effective, with somewhat higher (above, say 15%) being also satisfactory for use. Since a substantially 15% concentration of ethyl amine or its equivalent yields optimum results hereunder, a 5-15% range amount is preferred for use.

While the examples illustrate the invention as applied to the treatment of woven fabrics, yarns and staple, the invention has utility in modifying the properties of non-woven textiles. It has general application to any hydroxyl-containing derivative of cellulose, including commercial wood pulp, paper, cellulose, cellulose sponge, cupra-ammonium rayon, commercial cellulose acetate, mercerized cotton, and regenerated viscose in the form of fiber or cloth, etc. For example, cotton or rayon staple may be readily immersed in one of the organic conditioning agents mentioned, separated from the non-absorbed agent and immersed in the anhydrous liquid mixed metal ester composition. Thereafter, it is separated from the organic liquids, washed with water, and dried. During this operation the cellulose, whether it be cotton or a regenerated cellulose rayon, or a hydroxyl-containing derivative of cellulose, becomes modified by such composition to result in a cellulosic material containing from about 2% up to 40% or more of the mixed metals, calculated as oxides in chemical combination with the cellulose. Normally, the products of the invention will contain from about 5-35% of said metal oxides, and, preferably, from about 10-30% thereof. As noted, use has been had of elevated or boiling temperatures in the reaction of the metal esters with the cellulose material in the examples. However, this is not considered essential to the beneficial results of the invention. The reaction can be accomplished at lower temperatures through employment of longer contact times at the discretion of the operator. The temperature used in removal of solvents after completion of the reactions is likewise flexible, and one can employ any suitable vaporization conditions. The variable reaction times, temperature, pressure of the system when swelling and complexing as well as when reacting and tenderizing the swollen and complexed product by ester treatment, are as already indicated dependent upon the character of the initial cellulose material, the physical attributes of the swelling agent and the degree of subsequent metallization or degree of change of physical and chemical properties to be effected or desired.

Where relatively low-boiling liquids are used, such as anhydrous ammonia or methylamine, either low temperature operation at atmospheric pressure, or higher temperature operation at a pressure sufficient to maintain the major portion of ammonia derivative in the liquid state, is required. Short times of contact in both com-

plexing steps are also advantageous and effective. A minimum of about 30 minutes of contact is preferred in the first step, that is, in swelling and complexing the cellulose with the ammonia derivative; while a minimum of about 15 minutes is preferred in the second complexing or tenderizing step when addition and reaction of the ester with the complexed cellulose is effected. The reaction of the ester-ammonia-derivative-complexed cellulose intermediate with water depends on penetration, with a period of about 15 minutes to an hour at room temperature being preferably employed in this step.

The final product from this invention will advantageously contain not more than a trace of nitrogenous material and appreciable quantities of the titanium or zirconium and antimony. The relative amounts and total amounts of titanium and antimony present are not especially critical, but optimum results with respect to wool-like, wrinkle or crease resistant properties and resistance to photodegradation and dye fading will be found to occur when the finished, dried product contains between about 10 and 30% of the combined oxides,  $TiO_2$  and  $Sb_2O_3$ , and when such oxides are present in a weight ratio ranging from about .3 to 5. The preferred values lie roughly at 20% of combined oxides with approximately equal weights of  $TiO_2$  and  $Sb_2O_3$  present according to analysis. The mol ratio of  $MO_2/Sb_2O_3$ , therefore, lies in the range of about 1 to 10 and is preferably about 3 to 4, where M is either titanium or zirconium.

As indicated above, the invention yields a modified cellulosic textile material having the crease resistance and resilience approaching that of wool. Upon release after pressing, the fibers and textile will readily spring apart, a characteristic known as recovery. These attributes assure production of a material having desired loft (high bulk or volume for a given weight) properties which afford ready production of wool-like, open, porous fabrics of high covering power and thick, warm fabrics with a minimum of weight—qualities demanded in all apparel fabrics. Additionally, the product exhibits other improved characteristics noted, e.g., high resistance to photodegradation, mildew resistance, abrasion resistance, extensibility, elasticity and flame resistance, to afford a unique combination of properties which assure essential texture, warmth, fit, and durability characteristics which enhance its value for acceptance by textile manufacturers and the garment industry.

During the contemplated treatments and reaction, the strength of the cellulose material undergoing modification becomes poor and fabrics such as used in the examples lose strength to such an extent that they are easily damaged by punctures and tears. It is believed that the cellulose is degenerated under the conditions of the process by a breaking of the cross-linkage of cellulose. The antimony and titanium, or other metal, enters into chemical combination with the cellulose and the anhydrous product has poor strength due to this lack of cross-linkage between molecular units of the cellulose fiber. Upon treatment and regeneration with water, however, there is strong evidence that cross-linkage again takes place to cause the fabric to resume its original tensile strength. The cross-linkage at this time is believed to be somewhat different and a new chemical bonding takes place through the antimony and titanium or other treating metal which has entered into the complex structure. The improved properties are believed to be due in large measure to this new cross-linkage or bonding of both units of the cellulose structure. When subjected to normal washing treatment, the product will be found to be substantially nitrogen-free, indicating that a relatively pure metal-modified cellulosic material has been obtained.

That a chemical reaction and new chemical combination is obtained in the invention is readily evidenced from the results obtained when an alkyl antimonite and titanate are reacted with amine-swollen cellulose and measurement is undertaken of isopropanol liberated, in

accordance with the following procedure outlined in my concurrently filed copending application Serial No. 707,870, with all processing from the drying to the final product being effected under dry nitrogen to eliminate moisture pick-up.

The existence of a chemical combination of the treating metals with the cellulose is also evident from the excellent mildew resistance which the metallated, especially the antimonited and titanated cellulose product exhibits, as well as from the fact that such a result is not obtained when recourse to precipitation of  $TiO_2$  in a cellulosic fabric from an aqueous solution of compounds of the metals is undertaken.

I claim:

15. A method for preparing a cellulose textile material possessing substantially the single fiber, liveliness, crease resistance and bulk characteristics of wool, comprising reacting a cellulose textile material under anhydrous conditions in the presence of a nitrogenous chemical swelling agent for cellulose selected from the group consisting of ammonia and amine compounds which swell the cellulose and form nitrogenous complexes with the cellulose and containing a radical selected from the group consisting of  $-NH_2$  and  $>NH$ , with (1) a water hydrolyzable antimony ester corresponding to the formula  $(RO)_3Sb$  in which R is selected from the group consisting of a hydrocarbon and chlorinated hydrocarbon radical, and (2) a water hydrolyzable organic compound selected from the group consisting of
  - 20
  - 25
  - 30
  - 35
  - 40
  - 45
  - 50
  - 55
  - 60
  - 65
  - 70
  - 75
- (a) a metal ester corresponding to the formula  $Me(OR)_x$ , wherein Me is a metal selected from the group consisting of titanium, zirconium, hafnium, thorium, aluminum and iron and which forms a water-insoluble oxide and has a valence selected from the group consisting of 3 and 4 and has a coordination number in the oxide state at least one greater than the valence, R is selected from the group consisting of hydrocarbon and chlorinated hydrocarbon radicals, and x corresponds to the valence of the metal, and
- (b) a condensed ester of said hydrolyzable metal ester resulting from the reaction of said ester with water, continuing said reaction until a highly tendered metal ester-amine cellulose complex intermediate product forms of substantially reduced tensile and tear strength over that of the swollen cellulose textile obtained from said chemical agent treatment, contacting said metal ester-amine cellulose complex intermediate product with aqueous media consisting essentially of water which regenerates and restores said product to substantially the tensile strength of the original untreated cellulose textile material, and recovering the resulting chemically modified cellulose product.
2. A method for preparing a cellulose textile material possessing substantially the single fiber, liveliness, crease resistance and bulk characteristics of wool comprising reacting a cellulose textile material under anhydrous conditions in the presence of an alkyl amine chemical swelling agent for cellulose which swells the cellulose and forms nitrogenous complexes with cellulose, with (1) a water hydrolyzable antimony ester corresponding to the formula  $(RO)_3Sb$  in which R is selected from the group consisting of a hydrocarbon and chlorinated hydrocarbon radical, and (2) a water hydrolyzable organic titanium ester corresponding to the formula  $Ti(OR)_4$  in which R is selected from the group consisting of hydrocarbon and chlorinated hydrocarbon radicals, continuing said reaction until a highly tenderized metal ester-amine cellulose complex intermediate is obtained having a substantially reduced tensile and tear strength compared to the swollen cellulose textile obtained from said chemical agent treatment, subjecting said tenderized metal ester-amine cellulose complex intermediate to contact with aqueous media consisting essentially of water which regenerates and restores said cellulose intermediate to substantially the

tensile strength of the original untreated cellulose material, and recovering the resulting modified product containing in chemical combination with the cellulose from about 2% up to 40% of the metals of said esters, calculated as their oxides.

3. A method for preparing a cellulose textile material possessing substantially the single fiber, liveliness, crease resistance and bulk characteristics of wool comprising reacting a cellulose textile material under anhydrous conditions in the presence of an alkyl amine chemical swelling agent for cellulose which swells the cellulose and forms nitrogenous complexes with cellulose, with (1) a water hydrolyzable antimony ester corresponding to the formula  $(RO)_3Sb$  in which R is selected from the group consisting of a hydrocarbon and chlorinated hydrocarbon radical, and (2) a water hydrolyzable organic zirconium ester corresponding to the formula  $Zr(OR)_4$  in which R is selected from the group consisting of hydrocarbon and chlorinated hydrocarbon radicals, continuing said reaction until a highly tenderized metal ester-amine cellulose complex intermediate is obtained having a substantially reduced tensile and tear strength compared to the swollen cellulose textile obtained from said chemical swelling agent treatment, subjecting said tenderized cellulose complex intermediate to contact with aqueous media consisting essentially of water which regenerates and restores said cellulose intermediate to substantially the tensile strength of the original untreated cellulose material, and recovering the resulting modified product containing in chemical combination with cellulose from about 2% to 40% of the metals of said esters, calculated as their oxides.

4. A method for preparing a cellulose textile material possessing substantially the single fiber, liveliness, crease resistance and bulk characteristics of wool comprising swelling a cellulose textile material by treatment under anhydrous conditions with an alkyl amine chemical swelling agent for cellulose which forms nitrogenous complexes with cellulose, subjecting the resulting amine-treated, swollen and nitrogenous complexed cellulose product to reaction under anhydrous conditions with (1) a water hydrolyzable antimony ester corresponding to the formula  $(RO)_3Sb$  in which R is selected from the group consisting of a hydrocarbon and chlorinated hydrocarbon radical, and (2) a water hydrolyzable organic ester corresponding to the formula  $Me(OR)_x$  wherein Me is a metal selected from the group consisting of titanium, zirconium, hafnium, thorium, aluminum and iron and which forms a water-insoluble oxide and has a valence selected from the group consisting of 3 and 4 and a coordination number in the oxide state at least one greater than the valence, R is an alkyl radical, and x corresponds to the valence of the metal, continuing said reaction until a highly tendered metal ester-amine cellulose complex intermediate is obtained the tensile and tear strength of which is substantially reduced over that of the originally treated swollen cellulose textile, subjecting said cellulose complex intermediate product to contact with aqueous media consisting essentially of water which regenerates and restores said cellulose intermediate to substantially the tensile strength of the original untreated cellulose textile, and recovering the resulting modified cellulose product containing in chemical combination with the cellulose from about 5% to 35% of the metals of said esters, calculated as their oxides.

5. A method for preparing a cellulose textile material possessing substantially the single fiber, liveliness, crease resistance and bulk characteristics of wool, comprising immersing a cellulose textile material under anhydrous conditions in an alkyl amine chemical swelling agent for cellulose which forms nitrogenous complexes with cellulose until a swollen nitrogenous complexed cellulose product is obtained, removing under anhydrous conditions excess amine reactant from the swollen cellulose

product and immersing the latter for reaction under anhydrous conditions at temperatures ranging from about 25° C. to 150° C. in a solution of (1) a water hydrolyzable antimony ester corresponding to the formula  $(RO)_3Sb$  in which R is selected from the group consisting of a hydrocarbon and chlorinated hydrocarbon radical, and (2) a water hydrolyzable organic ester corresponding to the formula  $Me(OR)_x$  wherein Me is a metal selected from the group consisting of titanium, zirconium, hafnium, thorium, aluminum and iron and which forms a water-insoluble oxide and has a valence selected from the group consisting of 3 and 4 and a coordination number in the oxide state at least one greater than the valence, R is an alkyl radical, and x corresponds to the valence of the metal, until a highly tendered metal ester-amine cellulose complex intermediate is obtained with a tensile and tear strength substantially reduced over that of the amine-swollen cellulose textile, removing under anhydrous conditions excess of ester reactants from said tenderized intermediate and immersing said cellulose complex intermediate in aqueous media consisting essentially of water which regenerates and restores the intermediate to substantially the tensile strength of the original untreated cellulose textile and recovering the resulting modified cellulose product containing in chemical combination with the cellulose from about 5% to 35% of the metals of said esters, calculated as their oxides.

6. A method for preparing a cellulose textile material possessing substantially the single fiber, liveliness, crease resistance and bulk characteristics of wool, comprising immersing a cellulose textile material under anhydrous conditions in an alkyl amine chemical swelling agent for cellulose which forms nitrogenous complexes with cellulose, until a swollen nitrogenous complexed cellulose product is obtained, removing under anhydrous conditions excess amine reactant from said product and reacting the latter under anhydrous conditions at temperatures ranging from about 40° C. to 100° C. with an anhydrous solution of water hydrolyzable tributyl antimonite and water hydrolyzable titanium tetraisopropylate until a highly tendered metal ester-amine cellulose complex intermediate is obtained having a tensile and tear strength substantially reduced over that of the swollen cellulose textile, removing under anhydrous conditions excess unreacted antimonite and titanate from said cellulose complex intermediate and subjecting the latter to contact with water which regenerates and restores said intermediate to substantially the tensile strength of the original untreated cellulose textile material, and thereafter recovering the resulting chemically modified cellulose product.

7. A method for preparing a cellulose textile material possessing substantially the single fiber, liveliness, crease resistance and bulk characteristics of wool comprising immersing a cellulose textile material under anhydrous conditions in an alkyl amine chemical swelling agent for cellulose which forms nitrogenous complexes with cellulose, until a swollen nitrogenous complexed cellulose product is obtained, removing under anhydrous conditions excess amine reactant from said product and reacting the latter under anhydrous conditions at temperatures ranging from about 40° C. to 100° C. with a solution of water hydrolyzable tributyl antimonite and water hydrolyzable tetraisopropyl zirconate until a highly tendered metal ester-amine cellulose complex intermediate is obtained having a tensile strength and tear strength substantially reduced over that of the swollen cellulose textile, removing under anhydrous conditions excess unreacted antimonite and zirconate reactants from said cellulose complex intermediate and subjecting the latter to contact with water which regenerates and restores said intermediate to substantially the tensile strength of the original untreated cellulose textile material, and thereafter recovering the resulting chemically modified cellulose product.

8. A method for preparing a cellulose textile material

## 13

possessing substantially the single fiber, liveliness, crease resistance and bulk characteristics of wool, comprising immersing under anhydrous conditions a cellulose textile material in an alkyl amine chemical swelling agent for cellulose which forms nitrogenous complexes with cellulose until a swollen nitrogenous complexed cellulose product is obtained, removing under anhydrous conditions excess amine reactant from said product and reacting the latter under anhydrous conditions at temperatures ranging from about 40° C. to 100° C. with a solution of a water hydrolyzable alkyl ortho ester of antimony and water hydrolyzable alkyl ortho ester of iron until a highly tendered metal ester-amine cellulose complex intermediate is obtained having a tensile and tear strength substantially reduced over that of the swollen cellulose textile, removing under anhydrous conditions excess unreacted antimony and iron ester reactants from said cellulose complex intermediate and subjecting the latter to contact with water which regenerates and restores said intermediate to substantially the tensile strength of the original untreated cellulose textile material, and thereafter recovering the resulting chemically modified cellulose product.

9. A method for preparing a cellulose textile material possessing substantially the single fiber, liveliness, crease resistance and bulk characteristics of wool, comprising immersing a cellulose textile material under anhydrous conditions in an alkyl amine chemical swelling agent for cellulose which forms nitrogenous complexes with cellulose until a swollen nitrogenous complexed cellulose product is obtained, removing under anhydrous conditions excess amine reactant from said product and reacting the

## 14

latter under anhydrous conditions at temperatures ranging from about 40° C.-100° C., with a solution of a water hydrolyzable alkyl ortho ester of antimony and water hydrolyzable alkyl ortho ester of aluminum until 5 a highly tendered metal ester-amine cellulose complex intermediate is obtained having a tensile and tear strength substantially reduced over that of the swollen cellulose textile, removing under anhydrous conditions excess unreacted antimony and aluminum ester reactants from said cellulose complex intermediate and subjecting the latter to contact with water which regenerates and restores said intermediate to substantially the tensile strength of the original untreated cellulose textile material, and thereafter recovering the resulting chemically modified cellulose product.

## References Cited in the file of this patent

## UNITED STATES PATENTS

2,009,015 Powers \_\_\_\_\_ July 23, 1935  
2,525,049 Signaigo \_\_\_\_\_ Oct. 10, 1950

## FOREIGN PATENTS

517,464 Great Britain \_\_\_\_\_ Jan. 31, 1940

## OTHER REFERENCES

Balthis: Abstract No. 692,385, May 16, 1950.  
Speer: Ind. and Eng. Chem., February 1950, pp. 251-253.  
30 Gulledge: Ind. and Eng. Chem., March 1950, pp. 440-444.  
Moncrieff: Textile Colourist and Finisher, August 1950, pp. 394 and 395.